

Jan. 5, 1960

P. W. NEURATH

2,920,296

REDUCTION OF TRANSFORMER NOISE DUE TO MAGNETOSTRICTIVE EFFECTS

Filed Jan. 7, 1955



Inventor  
Peter W. Neurath,  
by Gilbert P. Tarleton  
His Attorney.

**REDUCTION OF TRANSFORMER NOISE DUE TO MAGNETOSTRICTIVE EFFECTS**

Peter W. Neurath, Lenox, Mass., assignor to General Electric Company, a corporation of New York

Application January 7, 1955, Serial No. 480,387

9 Claims. (Cl. 336—100)

The present invention relates to induction apparatus, and to the reduction of noise resulting from the operation thereof. More particularly, the invention relates to the treatment of magnetic material used in induction apparatus such as transformers to reduce their noise of operation due to magnetostrictive effects in the magnetic material.

It is well known that many materials when magnetized or demagnetized undergo changes in dimension, an effect called magnetostriction, which is defined as

$$\frac{\Delta L}{L}$$

or the change in length per unit length in the direction of magnetization under the magnetizing force applied. The magnetostrictive effect is an important factor in the manufacture of electrical induction apparatus, and particularly of power transformers, since it is a basic cause of the noise emanating from the transformers during normal operation.

The improvements in magnetic materials with respect to core loss and permeability which have been achieved in the past have made it feasible to operate transformers at higher induction than has been utilized heretofore. The magnitude of the magnetostrictive effect, however, and the noise resulting therefrom increase with the induction, and for this reason in many cases it has become necessary to design transformers to operate at lower inductions than that at which they would take full advantage of the otherwise excellent magnetic properties of the core material.

Various attempts have been made in the past to reduce such noise. One such attempt has involved abrading the surface of magnetic sheets in order to decrease the magnetostrictive effect, but this method was unsatisfactory in that abrasion was found to increase the watt losses of the magnetic material. Another method involving oxidation of the magnetic steel also resulted in high watt losses in the treated material. It has also been attempted to reduce magnetostrictive noise by employing core steel of increased silicon content, for example about 6%, but this has proved impractical due to the extreme brittleness of such a core material.

It is, therefore, an object of the present invention to reduce noise in induction apparatus such as transformers caused by magnetostrictive effects, while avoiding the above-mentioned disadvantages.

It is another object of the invention to provide magnetic materials having reduced magnetostrictive effects, and methods of producing such materials, so as to avoid noise caused thereby under induction conditions.

It is still another object of the invention to provide magnetic materials and a magnetic core assembly made therefrom for induction apparatus such as transformers wherein the magnetic materials are pre-tensioned to counteract compressive stresses encountered in the core assembly to reduce magnetostriction in the magnetic

materials to a minimum, thereby reducing the noise produced by the core assembly upon energization of the induction apparatus.

As a result of careful investigation on the phenomena of magnetostriction, particularly as applied to 3% oriented silicon steel sheet material, it has been found in accordance with the invention that the major cause of the present high noise level due to magnetostriction is the critical dependence of magnetostriction on stresses. 5 The magnetostrictive effects in magnetic steel can be increased six-fold by very slight compression of the sample, e.g., of about 300 pounds per square inch, which can be produced by bending a sample very slightly. Since magnetic sheet laminations are always bent appreciably when assembled into a transformer core under the usual manufacturing methods, the transformers turn out to be noisy.

It has been found, for example, that 3% Si-Fe transformer core sheet material of .012 inch and 0.14 inch thickness is quite sensitive to compression in the effects produced on magnetostriction. Compressive stress of the order of 1000 p.s.i. raises the magnetostriction from a strain free level of less than  $1 \times 10^{-6}$  (at 15,500 gauss) to a strained level of up to ten times that amount. Such compressive stress is always encountered as a consequence of the assembly of laminations that are not absolutely flat, which is the case of the usual type of magnetic steel laminations used for transformer cores.

I have discovered that such adverse effects of compressive stresses on magnetostriction can be largely overcome by prestressing the magnetic sheet material in tension to a tensile stress value which is at least as high as the compressive stresses subsequently imposed during the assembly process. If, for example, an unstressed material of low magnetostriction is subjected to such a pretensioning stress and as a result has a state of tension after assembly, a low magnetostriction core is obtained.

The prestressing of the magnetic steel can be done 40 in various ways. However, it is desirable that the method used to be economical, that it have no adverse effects on the quality of the finished material (e.g., permeability or watt losses), and that it be compatible with insulation, space factor and oil contamination requirements.

A practical method of providing suitable pretensioning of magnetic steel which has been found effective is by coating the surfaces of the magnetic materials with a varnish or similar material and then subjecting the coated magnetic sheet to an annealing treatment. The coating is preferably applied on each side of the metallic sheet and is of suitable thickness to produce the desired degree of tension on the final magnetic strip before assembly.

This method of producing sufficient tensile stresses 55 in magnetic sheet materials to counteract compressive stresses produced in subsequent assembly of the sheet materials is a significant feature of the invention in providing a practical means of pre-tensioning. However, optimum results in reducing noise in the finally 60 assembled magnetic structure are produced in accordance with the invention by a combination of steps, including the above coating process, which assures low magnetostriction of the finally assembled cores. To this end, it is important to start with magnetic sheet material which has been properly annealed to develop the magnetic qualities of the material while giving it low magnetostriction. The thus annealed material is then subjected to an appropriate coating process as described herein to confer thereon a tensile stress of suitable amount, depending on the magnitude of the bending (compressive) stresses encountered in assembly. In conjunction with the above quality annealing and coating

steps, additional measures may be taken to control the amount of bending stresses produced on the sheet material by the final assembly, as described more fully herein.

The invention will be better understood from the following description and in view of the accompanying drawing in which:

Fig. 1 is a view in elevation of a transformer core assembly which may embody the present invention;

Fig. 2 is an enlarged fragmentary view in perspective of a lower corner of the transformer core assembly shown in Fig. 1; and

Fig. 3 graphically illustrates how magnetostriction in a steel sample may be reduced in accordance with the invention.

Referring now to the drawing, and particularly to Fig. 1, there is shown a transformer core assembly 1 having a plurality of vertical legs 2, and lower and upper yoke members 3, 3' across the bottom and top of the legs 2, the legs 2 and yoke members 3, 3' each being composed of a plurality of superimposed magnetic steel laminations 4. As more clearly shown in Fig. 2, bolts 5 passing through legs 2, and clamp members 6, 6' held by bolts 8, serve to keep the laminations in assembly, the bolts 5 as well as clamp members 6, 6' producing, by their pressure, compressive stresses on the laminations in the final assembly of the transformer core. Also, it will be noted that spacers 7 are provided between the clamps 6, 6' and the laminations of the lower yoke 3 to keep the latter in assembled condition, the spacers 7 likewise serving to produce a compressive stress on the laminations. The compressive stresses herein referred to as being a primary cause of increased magnetostriction in the final assembly of the core are the compressive stresses along the length of the laminations, that is, in the direction of the orientation of the magnetic grains and of the flux induced in the magnetic steel.

Referring now to the graph in Fig. 3, the curve shown is for a particular magnetic sheet sample magnetized to saturation. It should be noted that while the magnetostriction values shown are for saturation flux density, the curves produced at flux densities of less than saturation, e.g., 15,500 gauss, correspond in shape to that shown in the graph, the particular values of magnetostriction varying in accordance with the different flux densities. The curves for other samples with initially lower magnetostriction can be superimposed on the curve shown by simply shifting the origin of the stress scale.

It should be mentioned in connection with the graph that since the actual point of zero internal stress of the magnetic sheet material cannot be accurately determined, the zero stress point has been arbitrarily selected as shown for a better understanding of the principle involved in the invention. It is to be understood, therefore, that the tensile stress indicated in the graph is due to the initial anneal actually represents relief of internal compressive stress and is not strictly the net tensile stress exerted on the material. A properly initially annealed sample will start at a point G on the curve lower than  $4 \times 10^{-6}$  magnetostriction, and any tensile stress put on by the coating will displace the stress point on the magnetostriction curve to some point T. Subsequent compression, due to bending in assembly, will increase the magnetostriction and will move back up the curve to the final condition, e.g., to point F as shown in Fig. 3. It is this final point that must be controlled in order to keep the noise in the transformer to a minimum. It is clear that this final point F depends on the following three factors: (1) the starting magnetostriction point (G) of a properly annealed sample, (2) the amount of tension produced by the coating, and (3) the amount of subsequent bending due to the assembly conditions.

It should be noted that the curve shows magnetostriction in relation to total stress in the magnetic sample where the total stress is the sum of the externally applied stress and the effective internal stress. The latter de-

pends on the prior treatment of the sample before coating, and the point G indicates on the curve approximately the amount of internal stress of a sample annealed at approximately 1175° C. The increased tension shown on the graph by the tension arrow is produced in the particular instance shown by a coating of Sterling varnish about 0.3 mil thick on the sample. The compression arrow indicates an amount of bending stress which is typically produced in the transformer core assembly, and it will be seen that this amount of subsequent compressive stress has been more than adequately counteracted by the combined effects of proper annealing and external pre-tensioning of the sample due to the coating. Improper annealing and/or an insufficient amount of pre-tensioning on the sample will cause the ultimate compressive stress to bring the final point to the more nearly vertical portion of the curve, the sample thus being in a condition where very slight increases in bending stress will result in considerably greater magnetostriction and, consequently, greater noise from the transformer core assembly.

The temperature at which the initial anneal of the magnetic material is carried out has been found to greatly influence the resulting magnetostriction. After an anneal at 1000° C. such as has been commonly used heretofore, the magnetostriction values may range from 3 to  $20 \times 10^{-6}$  at saturation flux density with an average value approximately as indicated by point A on the graph. If a higher temperature of annealing is used, e.g., 1100° C., a much smaller range of magnetostriction values will be found, with an average of approximately the amount indicated by point B on the curve. The annealing temperature which has been found to give the lowest magnetostriction while still producing optimum magnetic properties in the steel is in the range of 1100° C. and up, with 1175° C. preferred, and the state of magnetostriction of samples thus annealed is indicated by point G on the graph.

Coatings which have been found particularly suitable in accordance with the invention for producing tension on the samples are generally of a phosphate composition, and more specifically the coatings may be formed from a mixture of at least one refractory oxide and phosphoric acid in water. The following are two particular coating compositions found especially suitable, the proportions being given in parts by weight:

| C-10                                 |       |
|--------------------------------------|-------|
|                                      | Parts |
| MgO (USP heavy) -----                | 3.9   |
| H <sub>3</sub> PO <sub>4</sub> ----- | 38.2  |
| H <sub>2</sub> O -----               | 57.9  |
| <i>Sterling varnish</i>              |       |
|                                      | Parts |
| S <sub>1</sub> O <sub>2</sub> -----  | 16.0  |
| Fe <sub>2</sub> O <sub>3</sub> ----- | 28.7  |
| Al <sub>2</sub> O <sub>3</sub> ----- | 13.17 |
| P <sub>2</sub> O <sub>5</sub> -----  | 29.89 |
| H <sub>2</sub> O -----               | 50.17 |

Other coating compositions found suitable include aluminum phosphate, Al<sub>2</sub>O<sub>3</sub>:3P<sub>2</sub>O<sub>5</sub>, with the ratio of aluminum oxide to phosphorus pentoxide varying from 1:3 to 2:3. The following compositions in aqueous solution are illustrative of this type of coating material, the proportions being in parts by weight:

|                                      | I    | II   |
|--------------------------------------|------|------|
| Al <sub>2</sub> O <sub>3</sub> ----- | 8.6  | 12.8 |
| P <sub>2</sub> O <sub>5</sub> -----  | 33.1 | 33.9 |

The amount of water in the above compositions may be varied to give different consistencies of the mixture and to produce different thicknesses in the final coating. The coating may be applied in any suitable manner, as by spraying, dipping, brushing, or the like. After the

coating is applied, the coated sheet material is preferably heated to about 790° to firmly bind the coating to the surface of the metal. If residual internal stresses are present in the coated metal, due, for example, to cutting of the metal into laminae or to too rapid cooling after the initial quality anneal, or for any other reason, this anneal at 790° serves as a stress relief anneal to eliminate such internal stresses. For such purposes, the anneal is carried out at 790° C. in H<sub>2</sub> or N<sub>2</sub> gas or in air for about 8 hours as a batch anneal, or as a continuous anneal at the same temperature for a few minutes.

The following table illustrates the approximate amount of tension which may be produced in magnetic steel strips by Sterling varnish coatings of different thicknesses:

| Thickness of Sterling Varnish Coating, mils | Tension on Sample, p.s.i. |
|---------------------------------------------|---------------------------|
| .24                                         | 375                       |
| .30                                         | 420                       |
| .60                                         | 490                       |
| .90                                         | 975                       |

The above tension values were obtained where the coated samples were annealed in an H<sub>2</sub> atmosphere. It was found that even greater tension is produced by the same thicknesses of coating when the annealing was carried out in an atmosphere of N<sub>2</sub> or in air.

The range of thickness of the coating is preferably between 0.2-1.0 mil, this range of thickness producing tension of between 300 and 1400 p.s.i. Sterling varnish is preferable for the greater thicknesses, since the C-10 composition is not easily applied in thicknesses over 0.3 mil. It has been found that thicknesses of the coating over 1.0 mil do not produce added benefits in terms of increased tension or reduction in magnetostriction. Furthermore, too thick a coating is undesirable in that it takes up an excessive amount of space in the transformer core. Also, too great a thickness of the coating may cause breaking off of the coating due to concentration of compression at the interface between the coating and the metal surfaces, since the coating itself is subjected to longitudinal compression due to the tension it produces on the metal surface. Smaller thicknesses than the above range are not desirable since they do not produce the necessary amount of tension.

In order to test the magnetostrictive properties of the samples treated in accordance with the invention, the measurements were made with the samples curved to a predetermined radius of curvature. It was found that bending the samples to an 8 foot radius of curvature produced a compressive stress approximately equivalent to the amount of stress usually encountered in the assembly of the magnetic strips into a transformer core.

In a series of comparative magnetostrictive tests made on coated and uncoated Epstein strip samples (25 cm. x 3 cm. x .014 inch) annealed in H<sub>2</sub> at 1000° C. where the magnetostriction values were obtained with the samples bent to 8 and 16 foot radii of curvature, the following results were obtained:

| Coating of Sample                    | Tensile Stress, p.s.i. | Magnetostriction at 15,500-gauss (Average of 30 samples) |                       |
|--------------------------------------|------------------------|----------------------------------------------------------|-----------------------|
|                                      |                        | 8 ft. radius                                             | 16 ft. radius         |
| No coating                           | 150                    | $4.4 \times 10^{-6}$                                     | $0.9 \times 10^{-6}$  |
| C-10 (0.3 mils per side)             | 350                    | $1.9 \times 10^{-6}$                                     | $-0.1 \times 10^{-6}$ |
| Sterling Varnish (0.6 mils per side) | 640                    | $0.5 \times 10^{-6}$                                     | $-1.0 \times 10^{-6}$ |

From the above table it is evident that the magnetostriction of the coated samples was substantially reduced below that of the uncoated samples. Comparison of the values obtained as between the samples of 8 and 16 foot radii of curvature also shows that the greater the com-

pressive stress to which the samples are ultimately subjected, the more marked is the reduction of magnetostriction produced by the present coating process.

It will be apparent from the foregoing that the smaller the radius of curvature, the greater the compressive stress, and hence the greater the magnetostriction, in the magnetic strip. Since, as pointed out above, thicker coatings produce greater tensile stress for counteracting greater compressive stress, it is evident that in accordance with 10 the invention the thickness of the coating applied is inversely proportional to the radius of curvature of the strip.

As indicated previously, the final compressive stress to which the treated magnetic strips are subjected may be 15 controlled by additional measures and by thus restricting the compressive stresses, thinner coatings may be used to produce the requisite tension for counteracting the ultimate bending stresses. One method which may be used in conjunction with the coating process is the stress relief anneal already described. Another supplementary method is the process of heat flattening, already known by the art, which may be associated with the coating process and which consists generally in applying external tension to the strip while it is being heated to a suitable 25 temperature. By this method, the curvature of the strips may be reduced, so that in final assembly less bending stress will be encountered. A further measure is the so-called "in phase annealing" in which care is taken to nest the laminations during the stress relief anneal in the 30 same order that they will be assembled in the final core structure, so that the laminations, if they have any remaining curvature, will be curved in substantially the same direction in the final assembly and thus minimize compression due to bending stresses.

35 Any or all of the above supplementary measures may be used to control the bending stresses encountered. In this connection it might be noted that commercially produced annealed steel sheets are commonly classified in terms of radii of curvature to indicate the relative 40 amount of warping of the sheet. The present invention is of particular value in this regard, since it is only a simple matter to determine how much tension is necessary to be produced by the coatings applied (and hence the necessary thickness of the coating required) to overcome 45 the amount of bending stresses which would be expected by final assembly of a magnetic steel strip warped to the specified radius of curvature.

The following procedure is a particular process which 50 may be carried out in accordance with the present invention to provide low magnetostriction in transformer core laminations subjected to the usual assembly stresses. The magnetic steel material, which may be in coiled form and having an MgO separator coating on its surfaces, is subjected to a quality anneal at 1175° C. in dry hydrogen. 55 After cooling, the steel surface is cleaned, e.g., by light pickling and/or wire brushing. The steel is then coated with Sterling varnish to a thickness of about 0.3 mil per side and is then heat flattened to take out coil set and ripple. The material is then cut and batch annealed for 60 8 hours at 790° C. in N<sub>2</sub>.

These steps insure an adequate quality anneal, low 65 ripple, and a firmly adherent coating with good insulating qualities and which produces an average tension of at least 400 p.s.i. in the steel.

65 While 3% Si-Fe steel has been mainly referred to in describing the invention, primarily because this material is most commonly used at present as transformer core steel and appears to be most sensitive to compressive stresses in terms of increased magnetostriction, other 70 silicon-steel compositions or even pure iron can also be treated in accordance with the invention to produce lower magnetostriction. Thus, similar treatments of steel having up to 6% silicon content where the material is grain oriented is contemplated in accordance with the invention.

The present invention makes it possible not only to

reduce the magnetostriction of magnetic steel material in itself, but also, and more importantly, to provide low magnetostriction in the core structure as finally assembled, and it is the concept of the critical role played by the compressive stresses in assembly in increasing magnetostriction and the resulting noise which, so far as is known, has not been previously recognized in the art and which forms the basis of the present invention. This problem now having been recognized, the present invention provides effective, practical and economical measures to counteract and control such compressive stresses, and while producing these desirable results, it does not result in an increase of watt losses of the treated material, as is the case in prior art methods of reducing magnetostriction which rely solely on oxidation and abrading procedures.

Although the most practical method of producing tension in the steel strips is by the application of particular coatings as described above, other methods of applying tension could also be used, such as the following: application of a fused Pyrex, Vycor, or quartz coating at high temperature to produce tension upon cooling; a similar application of special low expansion glasses; plating, such as with  $\text{Cr}_2\text{O}_3$ , to produce tension; application of mechanical stress (tension) by the clamping structure of the core; and use of suitable porcelain enamels, ceramic coatings, or solution ceramics. Another possible method is the application at sub-zero temperatures of a suitable organic, inorganic or metallic coating such that on heating the strips up to ambient temperature a tension is produced therein.

Accordingly, the appended claims are intended to cover all such equivalent variations as come within the true spirit and scope of the invention.

What I claim as new and desire to secure by Letters Patent of the United States is:

1. A magnetic core assembly for induction apparatus comprising annealed grain-oriented magnetic sheet material; means holding said sheet material in assembly while exerting compressive stress thereon in the direction of grain-orientation of said sheet material; and means producing on said sheet material at least an amount of tension to fully counteract the compressive stress exerted by said holding means on said sheet material, whereby the magnetostriction of the sheet material and the consequent noise produced when the induction apparatus is energized are reduced.

2. A magnetic core assembly for induction apparatus comprising annealed grain-oriented magnetic sheet material; means holding said sheet material in assembly while exerting compressive stress thereon in the direction of grain-orientation of said sheet material; and means comprising a coating of a thickness of .2-1.0 mil on the surfaces of said sheet material for producing on said sheet material at least an amount of tension to fully counteract the compressive stress exerted by said holding means on said sheet material, whereby the magnetostriction of the sheet material and the consequent noise produced when the induction apparatus is energized are reduced.

3. A magnetic core assembly for transformers comprising a plurality of laminae of annealed magnetic strip material formed of a silicon-iron alloy containing up to 6% silicon; clamping means holding said laminae in assembly while exerting compressive stress thereon along their length; and a coating formed from a mixture of a least one refractory oxide and phosphoric acid in water and being of from .2-1.0 mil thickness on the surfaces of said laminae for producing on said magnetic strip material an amount of tension greater than required to fully counteract the compressive stress exerted by said clamping means on said strip material so as to leave a residual tension on the assembled strip material, whereby the magnetostriction of the strip material and the consequent noise produced when the transformer is energized are reduced.

4. A magnetic core assembly for transformers comprising a plurality of strips of annealed magnetic ma-

terial which are grain-oriented along their length and which in unassembled form have portions respectively bent to predetermined radii of curvature about axes transverse said strips; means holding said strips in assembly superimposed on each other in substantially flat condition while exerting compressive stress thereon along their length; and coating means of a thickness of .2-1.0 mil on at least said bent portions of said strips for producing tension therein counteracting the compressive stress exerted by said holding means, the thickness of said coating means on said bent portions being inversely proportional to their respective radii of curvature, whereby the magnetostriction of the strips and the consequent noise produced when the transformer is energized are reduced.

5. The method of reducing magnetostriction in magnetic sheet material adapted for use as core structure in induction apparatus wherein said magnetic sheet material is subjected to compressive stress in assembly in the induction apparatus, which method comprises annealing the magnetic sheet material for developing the magnetic properties and reducing the magnetostriction therein, and forming a coating of a thickness of .2-1.0 mil on the magnetic sheet material and heating the coated material to firmly bind the coating to the sheet material for producing at least an amount of tension on the thus annealed low magnetostriction magnetic sheet material to fully counteract the compressive stress encountered by said sheet material in assembly, whereby the magnetostriction of the sheet material and the consequent noise produced by the core assembly when the induction apparatus is energized are reduced.

6. The method of reducing magnetostriction in magnetic strip material adapted for use as core structure in induction apparatus wherein said magnetic strip material is subjected to compressive stress in assembly in the induction apparatus, which method comprises annealing the magnetic strip material for developing the magnetic properties and reducing the magnetostriction therein to less than  $4 \times 10^{-6}$  at saturation flux density, and forming a coating of a thickness of .2-1.0 mil on the magnetic strip material and heating the coated material to firmly bind the coating to the strip material for producing at least an amount of tension on the thus annealed low magnetostriction magnetic strip material to fully counteract the compressive stress encountered by said strip material in assembly, whereby the magnetostriction of the strip material and the consequent noise produced by the core assembly when the induction apparatus is energized are reduced.

7. The method of reducing magnetostriction in magnetic strip material adapted for use as core structure in induction apparatus wherein said magnetic strip material is subjected to compressive stress in assembly in the induction apparatus, which method comprises annealing the magnetic strip material for developing the magnetic properties and reducing the magnetostriction therein, and forming on the surfaces of the strip material a coating comprising a phosphate compound and having a thickness of from 0.2-1.0 mil, said coating being formed from a mixture of a phosphoric compound and at least one refractory oxide in water, and heating the coated material to firmly bind the coating to the strip material for producing an amount of tension on the thus annealed low magnetostriction magnetic strip material greater than required to fully counteract the compressive stress encountered by said strip material in assembly so as to leave a residual tension in the assembled strip material, whereby the magnetostriction of the strip material and the consequent noise produced by the core assembly when the induction apparatus is energized are reduced.

8. The method of reducing magnetostriction in magnetic strip material adapted for use as core structure in induction apparatus wherein said magnetic strip material is subjected to compressive stress in assembly in the in-

duction apparatus, which method comprises annealing the magnetic strip material for developing the magnetic properties and reducing the magnetostriction therein, applying on the surfaces of the strip material a coating comprising a mixture of a phosphoric compound and at least one refractory oxide in water, sufficient to provide a final coating .2-1.0 mil thick and subjecting the thus treated strip material to a second anneal at about 790° C. to relieve the internal stresses therein as well as to firmly bind the coating to the surfaces of the strip material and thereby produce by said coating at least an amount of tension on the thus treated magnetic strip material to fully counteract the compressive stress encountered by said strip material in assembly, whereby the magnetostriction of the strip material and the consequent noise produced by the core assembly when the induction apparatus is energized are reduced.

9. The method of reducing magnetostriction in silicon steel magnetic strip material adapted for use as core structure in induction apparatus wherein said magnetic strip material is subjected to compressive stress in final assembly in the induction apparatus, which method comprises annealing the magnetic strip material for developing the magnetic properties and reducing the magnetostriction therein, applying on the surfaces of the strip material a coating comprising a mixture of a phosphoric compound and at least one refractory oxide in water sufficient to provide a final coating .2-1.0 mil thick, sub-

jecting the thus treated magnetic material in the form of superimposed strips to a second anneal at about 790° C. for about 8 hours to relieve the internal stresses therein as well as to firmly bind the coating to the surfaces of the strips and thereby produce by said coating at least an amount of tension on the thus treated magnetic strips to fully counteract the compressive stress encountered by said strips in final assembly, and arranging the strips in final assembly in the same order and position in which they were arranged during said second anneal so as to reduce the bending stresses exerted during assembly, whereby the magnetostriction of the strips and the consequent noise produced by the core assembly when the induction apparatus is energized are reduced.

15

## References Cited in the file of this patent

## UNITED STATES PATENTS

|           |              |               |
|-----------|--------------|---------------|
| 1,857,215 | Ruder        | May 10, 1932  |
| 2,234,968 | Hayes et al. | Mar. 18, 1941 |
| 2,319,775 | Mittermaier  | May 18, 1943  |
| 2,394,047 | Elsey et al. | Feb. 5, 1946  |
| 2,467,868 | Somerville   | Apr. 19, 1949 |
| 2,484,242 | Nagel et al. | Oct. 11, 1949 |
| 2,492,095 | Gifford      | Dec. 20, 1949 |
| 2,494,349 | Mittermaier  | Jan. 10, 1950 |
| 2,501,349 | Nagel et al. | Mar. 21, 1950 |
| 2,501,846 | Gifford      | Mar. 28, 1950 |